



US010550513B2

(12) **United States Patent**  
**Zimmerman et al.**

(10) **Patent No.:** **US 10,550,513 B2**  
(45) **Date of Patent:** **Feb. 4, 2020**

(54) **FABRIC TREATMENT COMPOSITIONS AND METHODS**

(71) Applicants: **HBI Branded Apparel Enterprises, LLC**, Winston Salem, NC (US); **Cotton Incorporated**, Cary, NC (US)

(72) Inventors: **Keith Zimmerman**, Winston-Salem, NC (US); **Sha Fu**, Cary, NC (US); **Matthew J. Farrell**, Cary, NC (US)

(73) Assignees: **HBI Branded Apparel Enterprises, LLC**, Winston Salem, NC (US); **Cotton Incorporated**, Cary, NC (US)

(\*) Notice: Subject to any disclaimer, the term of this patent is extended or adjusted under 35 U.S.C. 154(b) by 0 days.

(21) Appl. No.: **16/013,583**

(22) Filed: **Jun. 20, 2018**

(65) **Prior Publication Data**

US 2018/0371689 A1 Dec. 27, 2018

**Related U.S. Application Data**

(60) Provisional application No. 62/523,619, filed on Jun. 22, 2017.

(51) **Int. Cl.**

**D06P 5/00** (2006.01)  
**D06P 3/60** (2006.01)

(Continued)

(52) **U.S. Cl.**

CPC ..... **D06P 5/002** (2013.01); **D06M 13/395** (2013.01); **D06M 15/227** (2013.01); **D06M 15/507** (2013.01); **D06P 3/6033** (2013.01)

(58) **Field of Classification Search**

CPC ..... D06P 5/002; D06P 1/5271; D06P 3/6033; D06P 3/54; D06P 3/52; D06M 3/395; D06M 5/507; D06M 4/227  
See application file for complete search history.

(56) **References Cited**

**U.S. PATENT DOCUMENTS**

3,762,872 A 10/1973 Acree  
3,853,459 A 12/1974 Harper et al.  
(Continued)

**FOREIGN PATENT DOCUMENTS**

EP 0474599 B1 4/1995  
GB 2259525 3/1993  
(Continued)

**OTHER PUBLICATIONS**

Beltrame et al., "Dyeing of Cotton in Supercritical Carbon Dioxide", Dyes and Pigments, vol. 39, Issue 4, Dec. 1, 1998, pp. 335-340.

(Continued)

*Primary Examiner* — Eisa B Elhilo

(74) *Attorney, Agent, or Firm* — Fish & Richardson P.C.

(57) **ABSTRACT**

A liquid fabric treatment composition including a hydrocarbon wax, a crosslinking agent, and a polyester warp sizing agent. The liquid fabric treatment composition may include a disperse dye. Methods of using these compositions for dyeing cellulose-containing fabric with a disperse dye include contacting a fabric containing cellulose with a liquid fabric treatment composition to yield a pretreated fabric, and heating the pretreated fabric to yield a treated fabric. The treated fabric contains a urethane compound formed by a reaction of the hydrocarbon wax, the crosslinking agent, and the cellulose of the fabric.

**22 Claims, 2 Drawing Sheets**



US 10,550,513 B2

Page 2

## FOREIGN PATENT DOCUMENTS

|    |              |         |
|----|--------------|---------|
| JP | 2003268682   | 9/2003  |
| WO | WO93/14259   | A1      |
| WO | WO94/09201   | A1      |
| WO | WO2004016849 | 2/2004  |
| WO | WO2006049504 | A2      |
| WO | WO2014005685 | A1      |
| WO | WO2014011278 | A9      |
| WO | WO2014133384 | A1      |
| WO | WO2016160771 | 10/2016 |

## OTHER PUBLICATIONS

“Ozcan et al., “Dyeing of Cotton Fibres with Disperse Dyes in Supercritical Carbon Dioxide”, *Dyes and Pigments*, vol. 36, Issue 2, Feb. 1998, pp. 103-110.”

International Search Report and Written Opinion in International Application No. PCT/US2018/038535, dated Sep. 13, 2018, 16 pages.

\* cited by examiner



FIG. 1



FIG. 2

## 1

## FABRIC TREATMENT COMPOSITIONS AND METHODS

## CROSS-REFERENCE TO RELATED APPLICATION

This application claims the benefit of U.S. Application No. 62/523,619 entitled "FABRIC TREATMENT COMPOSITIONS AND METHODS" and filed on Jun. 22, 2017, which is incorporated by reference herein in its entirety.

## TECHNICAL FIELD

This invention relates to liquid compositions for dyeing fibrous material.

## BACKGROUND

Dyeing fabric containing cellulosic fibers is an important chemical industrial process that results in commercial textile products. The natural fibers such as wool and silk, which are cationic polyamide (protein) fibers, are typically dyed using water-soluble acid dyes containing anionic groups such as residues of sulfuric, carboxylic, or phosphoric acids. Hydrophilic cellulosic fibers such as cotton, flax, and linen contain hydroxyl groups (—OH) and can be dyed using water-soluble dyes, such as direct (substantive) dyes or reactive dyes. Direct dyes physically bond to the hydrophilic fiber, e.g., by forming hydrogen bonds with the —OH groups of the cellulosic substrate. Reactive dyes chemically react with the fiber, e.g., by forming covalent bonds with the —OH groups of the cellulose. In some instances, reactive dyes can also be applied to protein fibers such as wool and silk and to some synthetic polyamides such as nylon. Acrylic fibers (made, e.g., from acrylonitrile) may be dyed using basic dyes. Hydrophobic synthetic fibers, such as polyester and acetate fibers, are typically dyed with disperse dyes that are sparingly water-soluble and do not have reactive or ionizable groups in their structure.

## SUMMARY

In a first general aspect, the present disclosure provides a liquid fabric treatment composition including a hydrocarbon wax; a crosslinking agent; and a polyester warp sizing agent.

In some embodiments, the liquid fabric treatment composition also includes an ultraviolet light inhibitor.

In some embodiments, the liquid fabric treatment composition also includes an anti-migrant.

In some embodiments, the liquid fabric treatment composition also includes a disperse dye.

In a second general aspect, the present disclosure provides a method of forming a liquid fabric treatment composition, the method including combining an aqueous solvent; a hydrocarbon wax, a crosslinking agent, and a polyester warp sizing agent, to form the liquid fabric treatment composition.

In some embodiments, the method also includes combining an ultraviolet inhibitor with the liquid fabric treatment composition.

In some embodiments, the method also includes combining an anti-migrant with the liquid fabric treatment composition.

In some embodiments, the method also includes combining a disperse dye with the liquid fabric treatment composition.

## 2

In some embodiments, the method also includes agitating the liquid fabric treatment composition to form a liquid dispersion.

In a third general aspect, the present disclosure provides 5 a method of treating fabric, the method including: (i) contacting fabric containing cellulose with a liquid dispersion to yield a pretreated fabric, wherein the liquid dispersion includes: a hydrocarbon wax; a crosslinking agent; and a polyester warp sizing agent; and (ii) heating the pretreated fabric to yield a treated fabric, wherein the treated fabric contains a urethane formed by a reaction of the hydrocarbon wax, the crosslinking agent, and the cellulose.

In some embodiments, the heating of the pretreated fabric includes reaching a temperature greater than a melting temperature of the hydrocarbon wax.

In some embodiments, the heating of the pretreated fabric includes drying the pretreated fabric at a temperature of at least 150° C. to obtain the treated fabric.

20 In some embodiments, a moisture content in the treated fabric is about 2 wt. % or less.

In some embodiments, the method of treating fabric also includes dyeing the treated fabric with a disperse dye.

25 In some embodiments, dyeing the treated fabric includes contacting the treated fabric with the disperse dye to yield a dyed fabric.

In some embodiments, dyeing the treated fabric includes jet dyeing the fabric.

30 In some embodiments, dyeing the treated fabric includes supercritical CO<sub>2</sub> (SCCO<sub>2</sub>) dyeing the fabric.

In some embodiments, the supercritical CO<sub>2</sub> (SCCO<sub>2</sub>) dyeing includes heating the treated fabric in a range of 120° C. to 130° C.

35 In some embodiments, dyeing the treated fabric includes sublimation printing.

In some embodiments, sublimation printing includes heating the treated fabric at a temperature in a range of 130° C. to 210° C.

40 In certain embodiments, the liquid dispersion contains a disperse dye. In some cases, the liquid dispersion includes an anti-migrant. In certain cases, the method of treating fabric includes thermosoling the treated fabric to yield a dyed fabric.

45 Implementations of the first, second, third, and fourth general aspects may include one or more of the following features.

In some embodiments, the composition is an aqueous dispersion.

In some embodiments, the hydrocarbon wax is in a form of a dispersion.

In some embodiments, the amount of hydrocarbon wax is in the range of about 1% on weight of goods ("o.w.g.") to about 10% o.w.g.

50 In some embodiments, the hydrocarbon wax is polyethylene wax.

In some embodiments, the polyethylene wax is oxidized.

In some embodiments, the polyethylene wax is anionic.

In some embodiments, the polyethylene wax contains carboxyl groups.

55 In some embodiments, the polyethylene wax is a high density polyethylene wax.

In some embodiments, a melting point of the polyethylene wax is in a range of about 100° C. to about 150° C.

60 In some embodiments, the crosslinking agent is in a form of a dispersion.

In some embodiments, the amount of the crosslinking agent is in the range of about 0.1% o.w.g. to about 5% o.w.g.

In some embodiments, the crosslinking agent contains nonionic blocked isocyanate.

In some embodiments, the crosslinking agent reacts with the hydrocarbon wax and a cellulose-containing fabric to form a urethane.

In some embodiments, the polyester warp sizing agent is in a form of a dispersion.

In some embodiments, the amount of the polyester warp sizing agent is in the range of about 1% o.w.g. to about 10% o.w.g.

In some embodiments, the polyester warp sizing agent is an anionic polyester warp size.

In some embodiments, the polyester contains sulfate moieties.

In some embodiments, the polyester contains sulfated isophthalic acid monomer units.

In some embodiments, the polyester contains sulfated terephthalic acid monomer units.

In some embodiments, an amount of the ultraviolet light inhibitor is in the range of about 0.1% o.w.g. to about 5% o.w.g.

In some embodiments, an amount of the anti-migrant is in the range from about 0.1% o.w.g. to about 10% o.w.g.

In some embodiments, the anti-migrant contains an acrylamide.

In some embodiments, an amount of the disperse dye in the composition is in the range from about 0.1% o.w.g. to about 10% o.w.g.

In some embodiments, the fabric is a garment.

The compositions and methods described herein allow disperse dyeing of cotton, for example, by applying sublimation printing, supercritical CO<sub>2</sub> dyeing, and thermosoling techniques to cotton substrates. A typical protocol for dyeing cotton with direct or reactive dyes involves the use of a large amount of water, salt, and energy, and generates significant amount of chemical waste. Disperse dyeing advantageously eliminates or decreases the consumption of water in the cotton dyeing processes. Furthermore, disperse dyeing is more efficient than the conventional cotton-dyeing processes. For example, disperse dyeing is a salt-free process that allows reuse of the dyebath and leaves less dye in the effluent. Also, disperse dyeing allows for application of luminescent dyes to cotton and yields colors that are not typically obtained on this type of fabric by conventional processes.

Methods and materials are described herein for use in the present application; other, suitable methods and materials known in the art can also be used. The materials, methods, and examples are illustrative only and not intended to be limiting. All publications, patent applications, patents, and other references mentioned herein are incorporated by reference in their entirety. In case of conflict, the present specification, including definitions, will control.

Other features and advantages of the present application will be apparent from the following detailed description and figures, and from the claims.

#### DESCRIPTION OF DRAWINGS

FIG. 1 is a flow chart for an exemplary method of pretreating a fabric with a liquid pretreatment composition to obtain a pretreated fabric, a dry pretreated fabric, an article of clothing prepared from a dry pretreated fabric, a fabric dyed with a disperse dye, or an article of clothing prepared from the dyed fabric.

FIG. 2 is a flow chart for an exemplary method of treating a fabric with a liquid treatment composition to obtain a

treated fabric, dry treated fabric, dyed fabric, or an article of clothing prepared from the dyed fabric.

#### DETAILED DESCRIPTION

5 Disperse dyes are an important class of dyes used in dyeing polyester fibers and other related materials such as nylon. Through their hydrophobic properties, these dyes are capable of penetrating into the similarly hydrophobic polyester fiber. The substantivity of the disperse dyes with respect to the polyester material allows for efficient diffusion of the disperse dyes into the polyester textiles. As used herein, the term "substantivity" refers to ability of a dye to be attracted by physical forces to a textile at the molecular level. The physical forces may include non-covalent bonding. Examples of non-covalent bonding include hydrogen bonds, electrostatic effects,  $\pi$ -effects, hydrophobic effects, and Van der Waals forces. The greater the attraction of the dye to the textile, the higher the substantivity of the dye to the textile.

10 Disperse dyes lack substantivity toward hydrophilic fibrous material and, therefore, disperse dyes are not typically used to dye cotton. The present disclosure provides liquid fabric treatment compositions that allow disperse dyeing of cotton. These compositions may be considered to be in two different general categories:

15 (1) pretreatment liquid compositions including a hydrocarbon wax, a crosslinking agent, and a polyester warp sizing agent. Such compositions may also contain an ultraviolet light inhibitor; and

20 (2) liquid fabric treatment compositions including a pre-treatment liquid composition of (1) and a disperse dye. Such compositions may also contain an anti-migrant.

25 Exemplary embodiments of the compositions, as well as the methods of making and using the compositions, are described herein. In one example, cotton fabric pretreated with the liquid composition of (1) may be further dyed with a disperse dye using conventional methods and apparatuses generally applicable to the disperse dyeing of polyester fabric, such as jet-dyeing. In another example, cotton fabric treated with the disperse dye-containing composition of (2) may be further thermosoled to provide the dyed cotton fabric.

#### Pretreatment Compositions

30 In some embodiments, the present disclosure provides a liquid fabric pretreatment composition including a hydrocarbon wax, a crosslinking agent, and a polyester warp sizing agent. Suitable examples of hydrocarbon waxes include oxidized high density polyethylene waxes. Suitable examples of crosslinking agents include blocked nonionic isocyanates. Suitable examples of polyester warp sizing agents include anionic polyester containing sulfated isophthalate or sulfated terephthalate monomer units. In some embodiments, the composition consists of a hydrocarbon wax, a crosslinking agent, and a polyester warp sizing agent. In other embodiments, the composition consists essentially of a hydrocarbon wax, a crosslinking agent, and a polyester warp sizing agent. In certain embodiments, the composition contains one or more additional components, as discussed herein. In one example, the composition includes an ultraviolet (UV) light inhibitor. Suitable examples of UV light inhibitors include benzophenone derivatives. In some embodiments, the composition is a liquid dispersion in an aqueous solvent. In one example, the composition is an aqueous dispersion.

35 As used herein, "dispersion" refers to a system consisting of particles of a dispersed phase (e.g., solid) and a continu-

ous phase (e.g., liquid). Where the particle size of the dispersed phase is greater than about 1  $\mu\text{m}$ , the dispersion is coarse, and where the particle size of the dispersed phase is between about 1 nm and 1  $\mu\text{m}$ , the dispersion is a colloid. An emulsion is a suitable example of a coarse dispersion where the dispersed phase and the continuous phase are both liquid.

#### Fabrics

In some embodiments, the fabric suitable for pretreatment is hydrophilic. In one example, the fabric contains a polysaccharide such as cellulose, which contains hydroxyl groups.

As used herein, the term “cellulose” or “cellulosic” refers to a complex polysaccharide molecule that is composed of disaccharide subunits containing two D-glucopyranoses joined by 1,4'- $\beta$ -glycoside bond (e.g., 4- $\beta$ -glucopyranosyl-D-glucopyranose).

As used herein, the term “hydroxyl” refers to an —OH moiety.

In some embodiments, the fabric contains at least one natural plant-based textile material. Suitable examples of natural plant-based textile material include cotton, linen, bamboo, hemp, jute and flax. In some embodiments, the fabric contains at least one natural animal-based textile material. Suitable examples of natural animal-based textile material include wool and silk.

In some embodiments, the fabric contains at least one synthetic fibrous material, for example, synthetic cellulosic fibrous material prepared from purified cellulose such as wood pulp. In one such example, the synthetic cellulosic fiber is rayon. Examples of rayon include viscose, modal, tensel, and lyocell. In another example, the synthetic fibrous material is polyester, polyamide, polyolefin, acrylonitrile, acrylic, or nylon. In some embodiments, the fabric is a blend of cellulosic fibrous material and synthetic material that does not contain cellulose. In one such example, the fabric is a blend of cotton and polyester. Suitable blends include 90/10, 80/20, 70/30, 65/35, 60/40, 50/50, 40/60, 35/65, 30/70, 20/80, and 10/90 cotton/polyester blends (w/w or v/v). In some embodiments, the fabric is a blend of cotton and viscose. Suitable examples of such blends include 90/10, 80/20, 70/30, 65/35, 60/40, 50/50, 40/60, 35/65, 30/70, 20/80 and 10/90 cotton/viscose blends (w/w or v/v). In some embodiments, the fabric is a blend of cotton and linen. Suitable examples of such blends include 90/10, 80/20, 70/30, 65/35, 60/40, 50/50, 40/60, 35/65, 30/70, 20/80 and 10/90 cotton/linen blends (w/w or v/v).

In some embodiments, the fabric contains cotton. In some embodiments, the fabric consists of cotton. In some embodiments, the fabric consists essentially of cotton. In some embodiments, the cotton contains from about 50 wt. % to about 100 wt. % cellulose.

Suitable ranges of cellulose in cotton include from about 60 wt. % to about 99 wt. %, from about 70 wt. % to about 95 wt. %, from about 75 wt. % to about 95 wt. %, from about 80 wt. % to about 95 wt. %, or from about 85 wt. % to about 95 wt. % cellulose. In some embodiments, cotton contains about 75 wt. %, about 80 wt. %, about 85 wt. %, about 90 wt. %, about 91 wt. %, about 92 wt. %, about 93 wt. %, about 94 wt. %, or about 95 wt. %

cellulose. In some embodiments, the weight of fabric containing cotton is from about 50 g/m<sup>2</sup> to about 300 g/m<sup>2</sup>, from about 60 g/m<sup>2</sup> to about 250 g/m<sup>2</sup>, from about 75 g/m<sup>2</sup> to about 200 g/m<sup>2</sup>, from about 100 g/m<sup>2</sup> to about 250 g/m<sup>2</sup>, or from about 125 g/m<sup>2</sup> to about 150 g/m<sup>2</sup>. In some embodiments, the weight of fabric containing cotton is about 125 g/m<sup>2</sup>, about 135 g/m<sup>2</sup>, about 140 g/m<sup>2</sup>, about 145 g/m<sup>2</sup>,

about 150 g/m<sup>2</sup>, about 155 g/m<sup>2</sup>, about 160 g/m<sup>2</sup>, about 165 g/m<sup>2</sup>, about 175 g/m<sup>2</sup>, about 200 g/m<sup>2</sup>, or about 250 g/m<sup>2</sup>.

In some embodiments, the cotton is bleached. In some examples, the cotton is bleached by any one of the conventional bleaching processes generally known in the art. In some embodiments, the cotton bleaching process is oxidative bleaching or reductive bleaching. In some embodiments, the bleached cotton is of commercial brightness.

In some embodiments, the cotton is raw cotton. In some 10 embodiments, the cotton is greige cotton. The yarn of the cotton greige typically contains natural seed oils, wax and seed pigments. In some examples, greige cotton contains less than about 5 wt. % or less than about 10 wt. % of cottonseed oils, wax, and pigments.

In some embodiments, the cotton is scoured. For example, 15 the cotton may be scoured by any one of the conventional scouring processes generally known in the art, using, for example, sodium carbonate and fabric detergent or liquid soap.

In some embodiments, the cotton is mercerized. For example, the cotton may be mercerized by any one of the conventional processes generally known in the art for mercerization of cotton, for example, by treating the cotton with sodium hydroxide followed by acidic treatment.

In some embodiments, the fabric is in the form of a woven 20 textile material, non-woven textile material, or knitted textile material. In some embodiments, the fibrous material is a yarn or a filament. In some embodiments, the fabric is woven, and the weave of the woven fabric is selected from plain, poplin, oxford, pinpoint, fil-a-fil, twill, herringbone, dobby, flannel, seersucker, and satin, or a combination thereof.

As used herein, the term “goods” refers to materials 25 prepared from the textile fibers. In one example, goods include woven or knitted cotton fabric.

#### Hydrocarbon Waxes

In some embodiments, the hydrocarbon wax in the fabric 30 pretreatment composition is an animal wax, a plant wax, or a petroleum-derived wax. As used herein, “wax” refers to a ductile hydrophobic material that is solid at room temperature and has a melting point of at least about 35° C.

In some embodiments, the hydrocarbon wax in the fabric 35 pretreatment composition is a petroleum-derived wax. One example of a petroleum-derived wax is paraffin wax. In some embodiments, the hydrocarbon wax contains long-chain hydrocarbons, such as alkanes and alkenes. In some embodiments, the hydrocarbon wax contains paraffins. Suitable examples of paraffins in the hydrocarbon wax include hentriacontane (C<sub>31</sub>H<sub>64</sub>). In certain embodiments, the hydrocarbon wax can contain one or more additional components. Examples of additional components in the hydrocarbon wax include fatty acids, fatty alcohols, and fatty esters. In some embodiments, the hydrocarbon wax contains esters of triacontanol and palmitic acid, cetyl palmitate, myricyl cerotate, lanolin, or mixtures thereof.

In some embodiments, the melting point of the hydrocarbon 45 wax is in a range of about 40° C. to about 250° C., about 50° C. to about 250° C., about 60° C. to about 200° C., about 75° C. to about 185° C., about 100° C. to about 150° C., or about 120° C. to about 160° C.

In some embodiments, the hydrocarbon wax contains a 50 polyolefin (polyalkylene). In some embodiments, the polyolefin is a copolymer or homopolymer of ethylene, propylene, 1-butene, 4-methyl-1-pentene, 3-methyl-1-butene, 4,4-dimethyl-1-pentene, 3-methyl-1-pentene, 4-methyl-1-hexene, 5-ethyl-1-hexene, 6-methyl-1-heptene, 1-hexene, 1-heptene, 1-octene, 1-nonene, 1-decene, and the like. In

some examples, the polyalkylene is polypropylene or polyethylene. In some embodiments, the polyalkylene is linear or branched. For example, the polyalkylene can have from 2 to 100 termini (e.g., from 2 to 5, 4 to 6, 5 to 6, or 3 to 6 termini). In some embodiments, the polyalkylene is linear and therefore has 2 termini.

In some embodiments, the hydrocarbon wax consists of a polyethylene wax. In some embodiments, the hydrocarbon wax consists essentially of a polyethylene wax. In such embodiments, the polyethylene wax contains compounds of formula  $(CH_2)_nH_2$ , wherein n ranges from 20 to 200. Polyethylene wax may also include copolymers of ethylene with butene, hexene, octane, or other monomers that co-polymerize with ethylene to form polyethylene. In some embodiments, the polyethylene is homopolyethylene. In some embodiments, the polyethylene wax is a low density, linear low density, medium density, or high density wax. As used herein, “low density polyethylene” refers to polyethylene having a density from about 0.91 g/cm<sup>3</sup> to about 0.93 g/cm<sup>3</sup>; “medium density polyethylene” refers to polyethylene having a density from about 0.93 g/cm<sup>3</sup> to about 0.94 g/cm<sup>3</sup>; “high density polyethylene” refers to polyethylene having a density from about 0.94 g/cm<sup>3</sup> to about 0.97 g/cm<sup>3</sup>. The low density, medium density, and high density polyethylene may be linear or branched. Linear polyethylene has 2 termini, while suitable examples of branched polyethylene include 2 to 5, 4 to 6, 5 to 6, or 3 to 6 termini.

In some embodiments, the polyethylene is high-density polyethylene (HDPE). In some embodiments, a density of the polyethylene in the composition ranges from about 0.91 g/cm<sup>3</sup> to about 1.2 g/cm<sup>3</sup>, from about 0.92 g/cm<sup>3</sup> to about 1.1 g/cm<sup>3</sup>, from about 0.93 g/cm<sup>3</sup> to about 0.97 g/cm<sup>3</sup>, from about 0.93 g/cm<sup>3</sup> to about 1.05 g/cm<sup>3</sup>, from about 0.93 g/cm<sup>3</sup> to about 0.99 g/cm<sup>3</sup>, from about 0.93 g/cm<sup>3</sup> to about 0.98 g/cm<sup>3</sup>, or from about 0.93 g/cm<sup>3</sup> to about 0.97 g/cm<sup>3</sup>. The density of polyethylene may be measured, for example, according to ASTM D 1505-68. In some embodiments, the polyethylene wax has a molecular weight in the range of from about 100 g/mol to about 20,000 g/mol, from about 400 g/mol to about 15,000 g/mol, from about 600 g/mol to about 10,000 g/mol, or from about 800 g/mol to about 8,000 g/mol.

In some embodiments, the hydrocarbon wax is oxidized. Oxidation of the hydrocarbon wax may be carried out by any method generally known in the art. In one example, the oxidation procedure involves passing an oxygen-containing gas into or over the hydrocarbon wax in a solid or melted form at elevated temperature. Suitable examples of an oxygen-containing gas include oxygen, ozone, and mixtures thereof. In some embodiments, a catalyst may be used in the oxidation process. One example of a suitable catalyst is metallocene. Oxidation of the hydrocarbon generally leads to breakdown of the hydrocarbon backbone and formation of carboxyl functional groups on the wax. In some embodiments, the oxidized hydrocarbon wax is anionic. The degree of oxidation of the wax may be determined by the acid number of the product. As used herein, “acid number” refers to a number of milligrams of KOH required to neutralize 1 gram of the material (e.g., oxidized wax or an anionic polyester). In some embodiments, the oxidized hydrocarbon wax has an acid number from about 5 to about 50, from about 10 to about 40, from about 10 to about 35, from about 10 to about 30, or from about 14 to about 22.

In some embodiments, the oxidized hydrocarbon wax is emulsifiable (e.g., the carboxyl groups on the wax provide emulsifiability). That is, the oxidized wax may be combined with an aqueous solvent to form an emulsion by a process known in the art, such as a water-on-wax technique or a

wax-on-water technique. The amount of water in the emulsion varies from about 10 wt. % to about 90 wt. %, from about 50 wt. % to about 70 wt. %, from about 60 wt. % to about 65 wt. %, or from about 10 wt. % to about 30 wt. %. In some embodiments, the amount of water in the hydrocarbon wax emulsion is about 20 wt. %. In other embodiments, the amount of water in the hydrocarbon wax emulsion is about 80 wt. %. In some embodiments, a base is added to the oxidized hydrocarbon wax prior to forming an emulsion, such that at least 25% of the carboxyl groups in the oxidized wax are converted to carboxylate ions. The base may be selected from NaOH and KOH. The amount of the base may range from about 1 wt. % to about 10 wt. %, from about 1 wt. % to about 8 wt. %, from about 2 wt. % to about 6 wt. %, or from about 3 wt. % to about 4 wt. %. One or more surfactants may also be combined with the emulsion.

In some embodiments, the hydrocarbon wax in the fabric pretreatment composition is an oxidized high density polyethylene wax. In such embodiments, the wax readily forms a dispersion when mixed with water. One example of such wax is Turpex ACN (available from Huntsman).

In some embodiments, after a fabric (e.g., cotton) is treated with the pretreatment composition, the hydrocarbon wax, when heated at or above the melting temperature of the wax, melts into the fabric and non-covalently binds to the fibers. Hydrocarbon wax has the long hydrocarbon chains, to which the hydrophobic disperse dyes may be substantive. In some embodiments, the long hydrocarbon chains in the wax promote the diffusion of the disperse dyes into the wax. Hydrocarbon wax is an amorphous material and is thus receptive to the disperse dye molecules. In some embodiments, the hydrocarbon wax in the pretreatment composition makes the fabric amenable to dying with disperse dyes.

#### Polyester Warp Sizing Agents

As used herein, the term “warp sizing” refers to a process of applying a protective adhesive coating upon the surface of a fabric to maintain good fabric quality by increasing smoothness, elasticity, frictional resistance, and absorbency of the fabric. A warp sizing agent is typically applied to textile strands or yarns to allow for smooth handling of the material during fabric formation processes such as weaving, to avoid damage to the textile. Natural hydrophilic fibers such as cotton may be sized using various hydrophilic polysaccharides such as starch, dextrin, carboxymethyl cellulose, hydroxyethyl cellulose, guar gum, alginates, and the like. These sizing agents are typically not suitable for use with hydrophobic synthetic fibers (e.g., polyester). Rather, polymeric hydrophobic sizing agents (e.g., polyacrylates, polyamides, polyesters) are commonly used to warp size polyester textiles. Nevertheless, a polyester warp sizing agent may be advantageously used in the pretreatment composition of the present disclosure for application to hydrophilic fabric substrates.

In some embodiments, a polyester warp sizing agent in a fabric pretreatment composition may contain any polyester backbone generally known in the art. In one example, a polyester backbone is prepared by polymerizing a diol and a dicarboxylic acid, or a dicarboxylic acid salt and an ester. In some embodiments, the diol may be a compound of formula HO—C<sub>1-6</sub>alkylene-OH, a compound of formula HO—C<sub>1-6</sub> haloalkylene-OH, a compound of formula HO—C<sub>3-7</sub>cycloalkylene-OH, or a compound of formula HO—C<sub>6-12</sub>arylene-OH. As used herein, “alkylene” or “C<sub>n-m</sub>alkylene” are used interchangeably and refer to a divalent alkyl (e.g., C<sub>n-m</sub>alkyl) linking group having n to m carbons (where n and m are independently selected from 1 to 10). The alkylene group may be linear or branched. Examples of

alkylene groups include, but are not limited to, methylene, ethan-1,1-diyl, ethan-1,2-diyl, propan-1,1-diyl, propan-1,3-diyl, propan-1,2-diyl, butan-1,4-diyl, butan-1,3-diyl, butan-1,2-diyl, 2-methyl-propan-1,3-diyl, and the like. In some embodiments, the alkylene moiety contains 2 to 6, 2 to 4, 2 to 3, 1 to 6, 1 to 4, or 1 to 2 carbon atoms. The term "haloalkylene" refers to an alkylene group in which one or more of the hydrogen atoms are replaced with a halogen atom (e.g., F, Cl, Br or I). Examples of haloalkylene group include difluoromethylene, tetrafluoroethylene and the like.

As used herein, the terms "cycloalkylene" and "C<sub>n-m</sub>cycloalkylene" are used interchangeably and refer to divalent non-aromatic cyclic hydrocarbons including cyclized alkyl or alkenyl linking groups having n to m carbons (where n and m are independently selected from 3 to 10). Cycloalkylene groups can include mono- or polycyclic (e.g., having 2, 3, or 4 fused rings) groups and spirocycles. Ring-forming carbon atoms of a cycloalkylene group can be optionally substituted by oxo or sulfido (e.g., C(O) or C(S)). Also included in the definition of cycloalkylene are moieties that have one or more aromatic rings fused to (i.e., having a bond in common with) the non-aromatic cyclic hydrocarbon, for example, benzo or thienyl derivatives of cyclopentane, cyclohexane, and the like. A cycloalkylene group containing a fused aromatic ring can be attached through any ring-forming atom including a ring-forming atom of the fused aromatic ring. Cycloalkylene groups can have 3, 4, 5, 6, 7, 8, 9, 10, 11, or 12 ring-forming atoms. In some embodiments, the cycloalkylene is a 3-12 membered monocyclic or bicyclic cycloalkylene. In some embodiments, the cycloalkylene is a C<sub>3-7</sub> monocyclic cycloalkane-diyl. Example cycloalkylene groups include cyclopropane-1,2-diyl, cyclobutane-1,2-diyl, cyclobutane-1,3-diyl, cyclopentane-1,2-diyl, cyclopentane-1,3-diyl, cyclohexane-1,2-diyl, cyclohexane-1,3-diyl, cyclohexane-1,4-diyl, cycloheptylene, cyclopentenylene, cyclohexenylene, cyclohexadienylene, cycloheptatrienylene, norbornylene, norpinylene, norcarnylene, and the like. In some embodiments, cycloalkylene is cyclopropane-1,2-diyl, cyclobutane-1,2-diyl, cyclobutane-1,3-diyl, cyclopentane-1,2-diyl, cyclopentane-1,3-diyl, or cyclohexane-1,2-diyl. In some embodiments, the cycloalkylene is a 3-8 membered or 3-7 membered monocyclic cycloalkylene group (e.g., C<sub>3-8</sub> or C<sub>3-7</sub> cycloalkylene). In some embodiments, the cycloalkylene is an 8-12 membered bicyclic cycloalkylene. In some embodiments, the 8-12 membered bicyclic cycloalkylene is an 8-12 membered fused cycloalkylaryl-diyl group (such as indane-1,2-diyl) or a 8-12 membered fused cycloalkylheteroaryl-diyl group.

As used herein, the terms "arylene" and "C<sub>n-m</sub> arylene" are used interchangeably and refer to a divalent aromatic hydrocarbon group, which may be monocyclic or polycyclic (e.g., having 2, 3 or 4 fused rings or rings connected by a single covalent bond), where n and m are independently selected from 6 to 20. Arylene groups include, e.g., phenylene, naphthylene, anthracenylene, phenanthrenylene, indanylene, indenylene, and the like. In some embodiments, arylene groups have from 6 to about 20 carbon atoms, from 6 to about 15 carbon atoms, or from 6 to about 10 carbon atoms. In some embodiments, the arylene group is phenylene. In some embodiments, the arylene group is biphenylene. In some embodiments, the arylene group is naphthylene.

In some embodiments, the diol is ethylene glycol (HO—CH<sub>2</sub>CH<sub>2</sub>OH), 1,4-butanediol (HO—(CH<sub>2</sub>)<sub>4</sub>—OH), bisphenol A, propylene-1,3-diyl (beta-propylene glycol, HO—(CH<sub>2</sub>)<sub>3</sub>—OH), resorcinol, methanediol (H<sub>2</sub>C(OH)<sub>2</sub>), (F<sub>3</sub>C)<sub>2</sub>

C(OH)<sub>2</sub>, propane-1,2-diol (alpha-propylene glycol, HO—CH<sub>2</sub>—CH(OH)—CH<sub>3</sub>), 2-methyl-2-propyl-1,3-propanediol, neopentyl glycol, 1,5-pentanediol, cyclohexane-1,2-diol (e.g., trans-1,2-cyclohexanediol, cis-1,2-cyclohexanediol), 1,2-cyclobutanediol, 1,3-cyclobutanediol, 2,2,4,4-tetramethyl-1,3-cyclobutanediol (CBDO), 1,2-cyclopropanediol, cyclopropane-1,1-diol, 1,2-cyclopentanediol, 1,3-cyclopentanediol, and the like. In some embodiments, the diol is ethylene glycol.

In some embodiments, the dicarboxylic acid may be a compound of formula HO—C(=O)—C<sub>1-6</sub> alkylene-C(=O)—OH, a compound of formula HO—C(=O)—C<sub>1-6</sub> haloalkylene-C(=O)—OH, a compound of formula HO—C(=O)—C<sub>3-7</sub> cycloalkylene-C(=O)—OH, or a compound of formula HO—C(=O)—C<sub>6-12</sub> arylene-C(=O)—OH. In some embodiments, the dicarboxylic acid is an aliphatic dicarboxylic acid such as adipic, sebacic, malonic, succinic, glutaric, pimelic, suberic, or azelaic acid. In some embodiments, the dicarboxylic acid is an aromatic dicarboxylic acid such as phthalic acid (o-phthalic acid), isophthalic acid (m-phthalic acid), terephthalic acid (p-phthalic acid), diphenic acid (biphenyl-2,2'-dicarboxylic acid), or 2,6-naphthalenedicarboxylic acid. In some embodiments, a salt or an ester of any one of the dicarboxylic acid compounds is used to prepare the polyester.

In some embodiments, any one of the diols or dicarboxylic acids described herein is substituted with 1, 2, 3, 4, or 5 moieties such as —S(=O)<sub>2</sub>—OH, —C(=O)—OH, and —P(=O)(OH)<sub>2</sub>. In some embodiments, the dicarboxylic acid is a compound of formula:



in which each R is independently —S(=O)<sub>2</sub>—OH, —C(=O)—OH, or —P(=O)(OH)<sub>2</sub>, or a salt or an ester of any one of these moieties, and x an integer of 1 to 4. In some embodiments, the dicarboxylic acid is a compound of formula:



or a salt (e.g., Na or K salt) or an ester (e.g., methyl or ethyl ester) thereof.

In some embodiments, a polyester warp sizing agent in a fabric pretreatment composition is polyethylene terephthalate (PET), polytrimethylene terephthalate, polyhexamethylene adipate diol (PHA), poly(1,4-butylene adipate) diol, poly(3-methyl pentamethylene) adipate diol (PMPA), or polyneopentyl adipate diol (PNA). In some embodiments, the polyester warp sizing agent in the fabric pretreatment composition is produced from ethylene glycol and at least one dicarboxylic acid component such as isophthalic acid, trimellitic anhydride, terephthalic acid, and 5-sulfoisophthalic acid, or a salt or an ester of any of these acids. In one example, the polyester warp sizing agent is prepared from ethylene glycol, isophthalic acid, and 5-sulfoisophthalic acid, or an ester or salt thereof. In some

## 11

embodiments, the polyester warp sizing agent in the fabric pretreatment composition includes anionic hydrophilic groups, such as sulfate groups. In one example, the polyester warp sizing agent contains sulfated isophthalic acid monomer units or sulfated terephthalic acid monomer units. In some embodiments, the polyester has an acid value of at least 5, at least 10, at least 20, or at least 30.

In some embodiments, the polyester warp sizing agent in the fabric pretreatment composition contains the maximum possible number of sulfated isophthalic acid groups in the polymer backbone. PW-600 (available from Ulterion) is a suitable example of a polyester that contains sulfated isophthalic acid groups in the polymer backbone.

After the fabric is treated with the pretreatment composition, the polyester warp sizing agent attracts the hydrophobic disperse dyes and enhances their ability to diffuse into the wax. The polyester binds to the hydrocarbon wax through hydrophobic interactions, thereby becoming non-covalently attached to the fabric.

## Crosslinking Agents

In some embodiments, the crosslinking agent is a compound capable of chemically reacting with the material from which the fabric is made, and with the hydrocarbon wax or with the polyester warp sizing agent, thereby covalently bonding the fabric with the wax or the polyester. In one example, the crosslinker is a compound of general formula:



where each RG is independently a reactive group such as  $-\text{OH}$ , halo,  $-\text{C}(\text{=O})\text{OH}$ ,  $-\text{C}(\text{=O})\text{Cl}$ ,  $-\text{S}(\text{=O})_2\text{OH}$ ,  $-\text{S}(\text{=O})_2\text{Cl}$ ,  $-\text{N}=\text{C}=\text{O}$ ,  $-\text{NH}_2$ ,  $-\text{CN}$ , or a similar reactive group; n and m is each independently an integer from 0 to 10 (e.g., 1, 2, 3, 4, 5, 6, or 7); and the -crosslinker-moiety is an alkylene, cycloalkylene, arylene, or a combination thereof. In one example, the -crosslinker-moiety is a combination of alkylene and arylene groups. Suitable examples of alkylene groups in the -crosslinker-moiety include optionally substituted methylene. Suitable examples of arylene groups in the -crosslinker-moiety include optionally substituted phenylene. In another example, the -crosslinker-moiety contains a polyalkylene glycol. Suitable examples of a polyalkylene alcohol in the -crosslinker-moiety include polyethylene glycol and polypropylene glycol. In some embodiments, the crosslinking agent in the fabric pretreatment composition is an isocyanate (e.g., polyisocyanate). In some embodiments, the isocyanate crosslinking agent contains at least one moiety of formula  $-\text{N}=\text{C}=\text{O}$ . In some embodiments, at least one moiety of formula  $-\text{N}=\text{C}=\text{O}$  is blocked, e.g., with an alcohol such as a polyol. The blocking may be achieved by reacting the isocyanate with an alcohol blocking agent under conditions known in the art. The reacting may be carried out until no free isocyanate groups are present. The blocking agents may be selected from alcohols such as methanol, ethanol, butanol, 2-butoxy ethanol, 2-(2-butoxyethoxy) ethanol, 2-hexoxyethanol, trimethylolpropane, ethylene glycol, propylene glycol, decyl alcohol, lauryl alcohol, and the like. In some embodiments, the crosslinking agent is 1,3-bis(1-isocyanato-1-methylethyl)benzene. In some embodiments, the 1,3-bis(1-isocyanato-1-methylethyl)benzene is blocked. In certain embodiments, the isocyanate crosslinker is blocked with a pyrazole.

In some embodiments, the crosslinking agent is nonionic. In some embodiments, the crosslinking agent is anionic.

In some embodiments, the crosslinking agent is 4,4'-diphenylmethane diisocyanate, toluene diisocyanate, hexamethylene diisocyanate (HDI), or a dimer, a trimer, or a

## 12

polymer thereof. In some embodiments, the crosslinking agent is a di- or triisocyanate. In some examples, the isocyanate crosslinker is at least one of tetramethylene diisocyanate, cyclohexane 1,3- and 1,4-diisocyanate-1-isocyanato-3,3,5-trimethyl-5-isocyanato-methylcyclohexane (isophorone diisocyanate, IPDI), methylene-bis(4-isocyanato)cyclohexane, triisocyanatononane, triphenylmethane 4,4'-diisocyanate, naphthylene-1,5-diisocyanate, 4-isocyanatotomethylloctane-1,8-diisocyanate (nonane triisocyanate, triisocyanatononane, TIN), and 1,6,11-undecane triisocyanate, or a dimer, a trimer, or a polymer of any of these compounds.

After the cotton fabric is treated with the pretreatment composition, the fabric is typically heated, for example, during the drying process. During the heating step, the blocking agent of the blocked isocyanate crosslinking agent is liberated, leaving the free isocyanate groups  $-\text{N}=\text{C}=\text{O}$ . These free isocyanate groups may react, for example, with the carboxyl groups of the oxidized hydrocarbon wax and the hydroxyl groups of the cellulose of the cotton fabric. The reaction of the isocyanate groups with the carboxyl groups of the wax and the hydroxyl groups of the fabric results in the formation of the covalent bonds, thereby increasing adhesion between the wax and the fabric. In some embodiments, the crosslinking agent reacts with the hydrocarbon wax and the cellulose-containing fabric to form a urethane, for example, as follows:



In some embodiments, the crosslinking agent in the fabric pretreatment composition is a nonionic blocked (poly)isocyanate. A suitable example of a nonionic blocked (poly)isocyanate includes Ruco-Coat FX 8041 (available from Rudolf Chemie).

## UV Light Inhibitors

In some embodiments, the fabric pretreatment composition contains an ultraviolet (UV) light inhibitor. In some embodiments, the UV light inhibitor is a benzophenone derivative, a benzotriazole derivative, a triazine derivative, or a mixture thereof. In some embodiments, the UV light inhibitor has a maximum absorbance ranging from 220 nm to 420 nm.

In some embodiments, the UV light inhibitor is a benzophenone derivative. Suitable examples of the benzophenone derivatives include 2,4-dihydroxybenzophenone, 2-hydroxy-4-methoxybenzophenone, 2-hydroxy-4-octyloxybenzophenone, 2-hydroxy-4-isooctyloxy benzophenone, 2-hydroxy-4-dodecyloxy benzophenone, 2,2'-dihydroxy-4-methoxybenzophenone, 2,2',4,4'-tetrahydroxybenzophenone, 2,2-dihydroxy-4,4'-dimethoxybenzophenone, 2-hydroxy-4-methoxy-5-sulfobenzophenone, and 2-hydroxy-4-benzylbenzophenone.

In some embodiments, the UV light inhibitor is a benzotriazole derivative. Suitable examples of the benzotriazole derivatives include 2-(2'-hydroxyphenyl) benzotriazole, 2-(2'-hydroxy-5-methylphenyl) benzotriazole, 2-(2'-hydroxy-3',5'-di-t-butylphenyl)-5-chlorobenzotriazole, 2-(2'-hydroxy-3'-sec-butyl-5'-methylphenyl) benzotriazole, 2-(2'-hydroxy-5'-octylphenyl) benzotriazole, 2-[2'-hydroxy-3',5'-(di-t-butyl) phenyl]benzotriazole, 2-[2'-hydroxy-3',5'-(di-t-amyl)phenyl]benzotriazole, 2-[2'-hydroxy-3',5'-di-( $\alpha,\alpha$ -

dimethylbenzyl)phenyl]benzotriazole, 2-(3'-t-butyl-2'-hydroxy-5'-methylphenyl)-5-chlorobenzotriazole, 2-(2'-hydroxy-3',5'-di-t-butyl)-5-chlorobenzotriazole, 2-(2'-hydroxy-5'-(1,1,3,3-tetramethylbutyl)phenyl) benzotriazole, 2-(2'-hydroxy-4'-octyloxyphenyl) benzotriazole, and 2-(2'-hydroxy-3',5'-di-t-amyl-phenyl) benzotriazole.

In some embodiments, the UV light inhibitor is a triazine derivative. Suitable examples of the triazine derivatives include 2,4,6-(triphenyl)-1,3,5-triazine, 2,4,6-tri(2-hydroxy-4-octyloxyphenyl)-1,3,5-triazine, 2-(2-hydroxy-4-hexyloxyphenyl)-4,6-bisphenyl)-1,3,5-triazine, 2-(2-hydroxy-4-octyloxyphenyl)-4,6-bis(2,4-dimethylphenyl)-1,3,5-triazine, 2-(2,4-dihydroxyphenyl)-4,6-bis(2,4-dimethylphenyl)-1,3,5-triazine, 2,4-bis(2-hydroxy-4-propyl-oxyphenyl)-6-(2,4-dimethylphenyl)-1,3,5-triazine, 2-[2-hydroxy-4-octyloxyphenyl)-4,6-bis(4-methylphenyl)-1,3,5-triazine, 2-(2-hydroxy-4-dodecyloxyphenyl)-4,6-bis(2,4-dimethylphenyl)-1,3,5-triazine, 2-(2-hydroxy-4-tridecyloxyphenyl)-4,6-bis(2,4-dimethylphenyl)-1,3,5-triazine, 2-[2-hydroxy-4-(2-hydroxy-3-octyloxypropoxy)-2-hydroxypropoxy]-4,6-bis(2,4-dimethyl-phenyl)-1,3,5-triazine, 2-(2-hydroxy-4-hexyloxyphenyl)-4,6-diphenyl-1,3,5-triazine, 2-(2-hydroxy-4-methoxyphenyl)-4,6-diphenyl-1,3,5-triazine, 2,4,6-tris[2-hydroxy-4-(3-butoxy-2-hydroxypropoxy)phenyl]-1,3,5-triazine, 2-(2-hydroxy-phenyl)-4-(4-methoxyphenyl)-6-phenyl-1,3,5-triazine, and 2-[2-hydroxy-4-(3-(2-ethylhexyl-1-oxy)-2-hydroxypropoxy)-2-hydroxypropoxy-phenyl]-4,6-bis(2,4-dimethylphenyl)-1,3,5-triazine.

After the fabric is treated with the pretreatment composition and then dyed with the disperse dye, the UV light inhibitor provides enhanced light fastness to the fabric. Suitable examples of the UV light inhibitors include Fadex ECS (available from Archroma).

#### Pretreatment Composition

As used herein, “o.w.g.” stands for “on weight of goods”.

In some embodiments, an amount of the hydrocarbon wax in the pretreatment composition is in a range from about 0.1% o.w.g. to about 50% o.w.g. about 0.5% o.w.g. to about 40% o.w.g., from about 1% o.w.g. to about 30% o.w.g., from about 1% o.w.g. to about 20% o.w.g., from about 1% o.w.g. to about 10% o.w.g., or from about 1% o.w.g. to about 5% o.w.g. In some embodiments, an amount of the hydrocarbon wax in the pretreatment composition is in a range from about 0.1 wt. % to about 50 wt. %, from about 0.5 wt. % to about 40 wt. %, from about 1 wt. % to about 30 wt. %, from about 1 wt. % to about 20 wt. %, from about 1 wt. % to about 10 wt. %, or from about 1 wt. % to about 5 wt. %. In some embodiments, amount of the hydrocarbon wax in the pretreatment composition is about 0.5 wt. %, about 1 wt. %, about 3 wt. %, about 5 wt. %, about 7 wt. %, about 10 wt. %, or about 20 wt. %.

In some embodiments, amount of the polyester warp sizing agent in the pretreatment composition is in the range from about 0.1% o.w.g. to about 50% o.w.g., from about 0.5% o.w.g. to about 40% o.w.g., from about 1% o.w.g. to about 20% o.w.g., from about 1% o.w.g. to about 10% o.w.g., or from about 1% o.w.g. to about 5% o.w.g. In some embodiments, amount of the polyester warp sizing agent in the pretreatment composition is in the range from about 0.1 wt. % to about 50 wt. %, from about 0.5 wt. % to about 40 wt. %, from about 1 wt. % to about 30 wt. %, from about 1 wt. %

to about 20 wt. %, from about 1 wt. % to about 10 wt. %, or from about 1 wt. % to about 5 wt. %. In some embodiments, amount of the polyester warp sizing agent in the pretreatment composition is about 0.5 wt. %, about 1 wt. %, about 3 wt. %, about 5 wt. %, about 7 wt. %, about 10 wt. %, or about 20 wt. %.

In some embodiments, an amount of the crosslinking agent in the pretreatment composition is in a range from about 0.01% o.w.g. to about 50% o.w.g., from about 0.05% o.w.g. to about 40% o.w.g., from about 0.1% o.w.g. to about 30% o.w.g., from about 0.1% o.w.g. to about 20% o.w.g., from about 0.1% o.w.g. to about 10% o.w.g., or from about 0.1% o.w.g. to about 5% o.w.g. In some embodiments, an amount of the crosslinking agent in the pretreatment composition is in a range from about 0.01 wt. % to about 50 wt. %, from about 0.05 wt. % to about 40 wt. %, from about 0.1 wt. % to about 30 wt. %, from about 0.5 wt. % to about 20 wt. %, from about 1 wt. % to about 10 wt. %, or from about 1 wt. % to about 5 wt. %. In some embodiments, an amount of the crosslinking agent in the pretreatment composition is about 0.1 wt. %, 0.5 wt. %, about 1 wt. %, about 1.5 wt. %, about 3 wt. %, about 5 wt. %, about 7 wt. %, about 10 wt. %, or about 20 wt. %.

In some embodiments, an amount of UV light inhibitor in the pretreatment composition is in a range from about 0.01% o.w.g. to about 50% o.w.g., from about 0.05% o.w.g. to about 40% o.w.g., from about 0.1% o.w.g. to about 30% o.w.g., from about 0.1% o.w.g. to about 20% o.w.g., from about 0.1% o.w.g. to about 10% o.w.g., or from about 0.1% o.w.g. to about 5% o.w.g. In some embodiments, an amount of UV light inhibitor in the pretreatment composition is in the range from about 0.01 wt. % to about 50 wt. %, from about 0.05 wt. % to about 40 wt. %, from about 0.1 wt. % to about 30 wt. %, from about 0.5 wt. % to about 20 wt. %, from about 1 wt. % to about 10 wt. %, or from about 1 wt. % to about 5 wt. %. In some embodiments, an amount of UV light inhibitor in the pretreatment composition is about 0.1 wt. %, about 0.5 wt. %, about 1 wt. %, about 1.5 wt. %, about 2 wt. %, about 2.5 wt. %, about 3 wt. %, about 5 wt. %, about 7 wt. %, about 10 wt. %, or about 20 wt. %.

In some embodiments, the pretreatment composition includes a hydrocarbon wax in an amount of about 1% o.w.g. to about 10% o.w.g., a polyester warp sizing agent in an amount of about 1% o.w.g. to about 10% o.w.g., and a crosslinking agent in an amount of about 0.1% o.w.g. to about 5% o.w.g. In some embodiments the pretreatment composition includes a hydrocarbon wax in an amount of about 1 wt. % to about 10 wt. %, a polyester warp sizing agent in an amount of about 1 wt. % to about 10 wt. %, and a crosslinking agent in an amount of about 1 wt. % to about 5 wt. %.

In some embodiments, the pretreatment composition contains an aqueous solvent. As used herein, the term “aqueous solvent” refers to a liquid containing at least 50%, at least 60%, at least 70%, at least 90%, or at least 95% water by volume. In some embodiments, the aqueous solvent is water. In some embodiments, the amount of the aqueous solvent in the composition is sufficient to produce a dispersion.

#### Optional Additives

In some embodiments, the fabric pretreatment composition contains at least one additive such as a dispersing agent, a surfactant, a plasticizer, a defoamer, a deflocculant, an emulsifier, a pH stabilizer, a wetting agent, a penetration enhancer, or an absorption enhancer. Any of the dispersing agents, surfactants, plasticizers, defoamers, deflocculants, emulsifiers, wetting agents, absorption and penetration enhancers generally known to be applicable in the dyeing

industry and capable of ensuring the stability of the aqueous dispersion may be used in a fabric pretreatment composition.

In some embodiments, the dispersing agent is anionic. In some embodiments, the dispersing agent is a lignosulfonate. In some embodiments, the dispersing agent is a surfactant, such as polyoxyethylenated straight chain alcohol, nonylphenolethoxylate, ethoxylated sorbitan monolaurate, or ethoxylated sorbitan monostearate. In some embodiments, the surfactant includes at least one of ARKOPAL N-300, BRU 30, BRU 35, BRIJ 56, BRU 58, EGE Coco, EGE No. 10, GENAPOL X-150, TERGITOL NP-10, MARLIPAL 013/90, PLURONIC PE6400, SAPOGENATT-300, T-MAZ 60K, T-MAZ 20, TRITON X-45, TRITON X-100, TRITON X-102, TRITON X-114, TRITON X-165, or TWEEN 80. In some embodiments, the surfactant includes at least one of sodium lauryl sulfate, cocamidopropyl betaine, ethoxylated nonylphenol, lauric acid diethanolamide, diethanolamine, polyethoxylated linear secondary alcohol, polyethoxylated tallow amine, poly(ethylene glycol) monooleate, and coconut oil monoethanolamide. In some embodiments, the fabric pretreatment composition is dispersant-free. In some embodiments, the emulsifier is a polyol such as propylene glycol, or an oleic acid sorbitan monoester.

In some embodiments, an amount of each additive in the fabric pretreatment composition is in a range from about 0.01% o.w.g. to about 50% o.w.g., from about 0.05% o.w.g. to about 40% o.w.g., from about 0.1% o.w.g. to about 30% o.w.g., from about 0.1% o.w.g. to about 20% o.w.g., from about 0.1% o.w.g. to about 10% o.w.g., or from about 0.1% o.w.g. to about 5% o.w.g. In some embodiments, an amount of the at least one additional ingredient in the pretreatment composition is in a range from about 0.01 wt. % to about 50 wt. %, from about 0.05 wt. % to about 40 wt. %, from about 0.1 wt. % to about 30 wt. %, from about 0.1 wt. % to about 20 wt. %, from about 0.1 wt. % to about 10 wt. %, from about 0.1 wt. % to about 5 wt. %, or from about 0.1 wt. % to about 1 wt. % (based on the weight of the composition). In some embodiments, an amount of each additive in the pretreatment composition is about 0.1 wt. %, about 0.5 wt. %, about 1 wt. %, about 1.5 wt. %, about 3 wt. %, or about 5 wt. %.

#### Fabric Treatment Disperse Dye-Containing Compositions

In some embodiments, the present disclosure provides a liquid fabric treatment composition containing a hydrocarbon wax, a crosslinking agent, a polyester warp sizing agent, and a disperse dye. In some embodiments, the liquid fabric treatment composition consists of an aqueous solvent, a hydrocarbon wax, a crosslinking agent, a polyester warp sizing agent, and a disperse dye. In other embodiments, the liquid fabric treatment composition consists essentially of a hydrocarbon wax, a crosslinking agent, a polyester warp sizing agent, and a disperse dye. In some embodiments, the composition includes an ultraviolet (UV) light inhibitor. In certain embodiments, the composition includes one or more optional additives. In one example, the composition includes an anti-migrant. In some embodiments, the composition is a liquid dispersion in an aqueous solvent (e.g., the composition is an aqueous dispersion).

Examples of fabrics suitable for treatment with the dye-containing composition, and examples of suitable hydrocarbon waxes, polyester warp sizing agents, crosslinking agents, UV light inhibitors, and optional additional additives include those described herein with respect to the pretreatment compositions.

#### Disperse Dyes

In some embodiments, the disperse dye in the fabric treatment composition is hydrophobic. In some embodiments, the disperse dye is nonionic. In some embodiments, the disperse dye has substantivity toward the hydrocarbon wax or the polyester warp sizing agent. In some embodiments, the disperse dye is water insoluble or sparingly water-soluble. In some embodiments, the disperse dye is used for dyeing fabric in the presence of a dispersing agent. 5 In some embodiments, the dye is free of a dispersant. In one example, a dispersant-free composition includes less than about 0.1 wt. % of a dispersant. In some embodiments, the dispersant-free composition includes less than about 0.01 wt. % of a dispersant. 10 In some embodiments, the disperse dye is a class A-D dye according to the ICI classification. In some embodiments, the disperse dye has low, medium, or high molecular weight. As used herein, the term "low molecular weight disperse dye" refers to a low energy disperse dye for dyeing fabric at 15 a temperature of at least 77° C. In some embodiments, the low molecular weight dyes are poorly resistant to sublimation. As used herein, the term "medium molecular weight disperse dye" refers to a medium energy disperse dye for dyeing fabric at a temperature in the range of about 104° 20 C.-110° C. In some embodiments, the medium molecular weight disperse dye provides better sublimation fastness than the low molecular weight dye. As used herein, the term "high molecular weight disperse dye" refers to a high energy dye for dyeing fabric at a temperature of at least 129° C. In 25 some embodiments, the high molecular weight dye is suitable for continuous dyeing and provides fastness properties superior to the fastness properties provided by the medium molecular weight dye.

In some embodiments, the disperse dye is a substituted 30 azo, anthraquinone, or diphenylamine compound. In some embodiments, the disperse dye is a nitroaryl amino disperse dye, a coumarin disperse dye, a methine disperse dye, a naphthostyryl disperse dye, a quinophthalone disperse dye, a formazan disperse dye, or a benzodifuranone disperse dye. 35 In some embodiments, a disperse dye of any color may be used in the present compositions.

Suitable examples of the azo disperse dyes include C.I. Disperse Yellow 3, C.I. Disperse Orange 25, C.I. Disperse Red 167, C.I. Disperse Violet 33, and C.I. Disperse Blue 79. 40 Suitable examples of the anthraquinone disperse dyes include C.I. Disperse Violet 4, C.I. Disperse Red 15, C.I. Disperse Red 60, and C.I. Disperse Violet 26.

In some embodiments, suitable examples of the disperse dyes include C.I. Disperse Red 92, C.I. Disperse Red 229, 45 C.I. Disperse Blue 60, C.I. Disperse Blue 87,

C.I. Disperse Blue 56, C.I. Disperse Yellow 114, C.I. Disperse Yellow 211, C.I. Disperse Yellow 54, C.I. Disperse Orange 30, C.I. Disperse Orange 31, C.I. Disperse Orange 44, C.I. Disperse Orange 61, C.I. Disperse Red 50, C.I. 50 Disperse Red 73, C.I. Disperse Red 82, C.I. Disperse Red 324, C.I. Disperse Red 356, C.I. Disperse Red 376, C.I. Disperse Red 382, C.I. Disperse Red 383, C.I. Disperse Violet 93, C.I. Disperse Violet 107, C.I.

Disperse Blue 56, C.I. Disperse Blue 93, Disperse Blue 60, C.I. Disperse Blue 183, C.I. Disperse Blue 284, C.I. Disperse Blue 291, C.I. Disperse Blue 337, C.I. Disperse Blue 354, C.I. Disperse Blue 378, C.I. Disperse Green 9, C.I. Disperse Green 6, C.I. Disperse Green 5, C.I. Disperse Green 1, and C.I. Disperse Green 2.

In some embodiments, the disperse dye is C.I. Disperse Red 92, C.I. Disperse Blue 79, C.I. Disperse Blue 291, or C.I. Disperse Orange 30.

## Dye-Containing Compositions

In some embodiments, the liquid dye-containing fabric treatment composition contains a hydrocarbon wax, a polyester warp sizing agent, a crosslinking agent, and optionally a UV light inhibitor in the amounts described herein with respect to the pretreatment compositions.

In some embodiments, an amount of disperse dye in the composition is in a range from about 0.01% o.w.g. to about 50% o.w.g., from about 0.05% o.w.g. to about 40% o.w.g., from about 0.1% o.w.g. to about 30% o.w.g., from about 0.1% o.w.g. to about 20% o.w.g., or from about 0.1% o.w.g. to about 10% o.w.g. In some embodiments, an amount of disperse dye in the composition is in a range from about 0.01 wt. % to about 50 wt. %, from about 0.05 wt. % to about 40 wt. %, from about 0.1 wt. % to about 30 wt. %, from about 0.5 wt. % to about 20 wt. %, from about 1 wt. % to about 10 wt. %, or from about 1 wt. % to about 5 wt. %. In some embodiments, an amount of disperse dye in the composition is about 0.1 wt. %, about 0.5 wt. %, about 1 wt. %, about 1.5 wt. %, about 2 wt. %, about 2.5 wt. %, about 3 wt. %, about 5 wt. %, about 7 wt. %, about 10 wt. %, or about 20 wt. % (based on the weight of the composition).

In some embodiments, a liquid dye-containing fabric treatment composition includes a hydrocarbon wax in an amount of about 1% o.w.g. to about 10% o.w.g., a polyester warp sizing agent in an amount of about 1% o.w.g. to about 10% o.w.g., a crosslinking agent in an amount of about 0.1% o.w.g. to about 5% o.w.g., and a disperse dye in an amount of about 0.1% o.w.g. to about 10% o.w.g. In some embodiments, a liquid dye-containing fabric treatment composition includes a hydrocarbon wax in an amount of about 1 wt. % to about 10 wt. %, a polyester warp sizing agent in an amount of about 1 wt. % to about 10 wt. %, a crosslinking agent in an amount of about 1 wt. % to about 5 wt. %, and a disperse dye in an amount from about 1 wt. % to about 10 wt. % (based on the weight of the composition).

## Optional Additives

In some embodiments, the liquid dye-containing fabric treatment composition optionally contains at least one additional ingredient. Exemplary additional ingredients and their amounts include those described herein with respect to the pretreatment compositions.

In some embodiments, the liquid dye-containing fabric treatment composition includes an anti-migrant. Anti-migrants promote uniform color distribution, inhibit dye migration during the dyeing process, and control the dye penetration into the fabric, film forming, and thickening, and impart non-tackiness to the dye composition. In some embodiments, the anti-migrant is a polyacrylic acid-based migration inhibitor or vinyl acetate-based migration inhibitor. In some embodiments, the anti-migrant contains an acrylamide. In some embodiments, the anti-migrant is sodium alginate based. In some embodiments, the anti-migrant is anionic, cationic, or nonionic. In some embodiments, the anti-migrant is suitable for thermosol dyeing of polyester fabric. In some embodiments, the anti-migrant is natural or synthetic. In some embodiments, the anti-migrant is carboxymethylcellulose, SOLIDOKOLL, guar gum, PMS-100 (acrylic acid copolymer), THERMOCOL MIN, THERMOCOL MP, or PRIMASOL FFAM.

In some embodiments, an amount of the anti-migrant in the composition is in a range from about 0.01% o.w.g. to about 50% o.w.g., from about 0.05% o.w.g. to about 40% o.w.g., from about 0.1% o.w.g. to about 30% o.w.g., from about 0.1% o.w.g. to about 20% o.w.g., from about 0.1% o.w.g. to about 10% o.w.g., or from about 0.1% o.w.g. to about 5% o.w.g. In some embodiments, an amount of the

anti-migrant in the composition is in a range from about 0.01 wt. % to about 50 wt. %, from about 0.05 wt. % to about 40 wt. %, from about 0.1 wt. % to about 30 wt. %, from about 0.5 wt. % to about 20 wt. %, from about 0.5 wt. % to about 10 wt. %, from about 0.5 wt. % to about 5 wt. %, or from about 0.5 wt. % to about 2 wt. %. In some embodiments, an amount of the anti-migrant in the composition is about 0.1 wt. %, about 0.5 wt. %, about 1 wt. %, about 1.5 wt. %, about 2 wt. %, about 2.5 wt. %, about 3 wt. %, or about 5 wt. % (based on the weight of the composition).

## Methods of Making the Compositions

## Pretreatment Composition

In some embodiments, a pretreatment composition is prepared by combining a crosslinking agent, a hydrocarbon wax, a polyester warp sizing agent, and an aqueous solvent in a reaction vessel. In some embodiments, combining the components includes agitation, stirring, or shaking. In some embodiments, the components are combined at room temperature.

In some embodiments, a crosslinking agent is combined with water to form a first mixture, followed by combining a hydrocarbon wax with the first mixture to form a second mixture, followed by combining a polyester warp sizing agent with the second mixture to form the pretreatment composition.

In other embodiments, a hydrocarbon wax is combined with water to form a first mixture, followed by combining a crosslinking agent with the first mixture to form a second mixture, followed by combining a polyester warp sizing agent with the second mixture to form the pretreatment composition.

In yet other embodiments, a polyester warp sizing agent is combined with water to form a first mixture, followed by combining a hydrocarbon wax with the first mixture to form a second mixture, followed by combining a crosslinking agent with the second mixture to form the pretreatment composition.

In some embodiments, combining the components is carried out for a length of time of about 5 minutes to about 2 hours. In some embodiments, a UV light inhibitor is further added to the pretreatment composition. In some embodiments, combining the components yields an aqueous dispersion. In some embodiments, the dispersion is stable. In one example, the dispersion is stable for at least 2-24 hours.

In some embodiments, each of the components of the pretreatment composition is combined in a form of an aqueous dispersion. In one example, an aqueous dispersion of a hydrocarbon wax, an aqueous dispersion of a crosslinking agent, an aqueous dispersion of a polyester warp sizing agent, and an aqueous dispersion of a UV light inhibitor are combined to yield the pretreatment composition.

## Dye-Containing Fabric Treatment Composition

In some embodiments, to prepare a dye-containing fabric treatment composition, a disperse dye is combined with a pretreatment composition prepared as described herein. In some embodiments, an anti-migrant is combined with a dye-containing fabric treatment composition. The combining may be carried out with agitation or stirring, at about room temperature. In some embodiments, the combining yields a stable dispersion.

## Methods of Treating Fabric

## Fabric Treatment with Pretreatment Compositions

FIG. 1 is a flow chart showing operations in exemplary process 100 for treating fabric with a pretreatment composition. In 102, fabric is contacted with a liquid pretreatment

composition to yield a wetted fabric. The terms "wet," "moisten," and "dampen" are used interchangeably.

In some embodiments, dampening the fabric with the pretreatment composition is carried out using conventional padding equipment. Suitable examples of the conventional padding equipment include vessels, apparatuses, and machinery used in batch fabric dyeing. In some examples, equipment used in the padding process includes at least one fabric batch roll, at least one pad liquor trough, squeezing mangles, and a dryer unit. In some embodiments, wetting the fabric with the pretreatment composition is carried out by providing the pretreatment composition to a pad liquor trough and padding the fabric with the liquor at about 100% wet pick-up.

As used herein, the term "wet pick-up" (WPU) refers to the ratio of the weight of the liquid composition picked up by the fabric to the weight of the dry fabric prior to contacting the fabric with the liquid composition. In some embodiments, WPU is expressed as a fraction of 100. For example, a WPU of 100% refers to a 1/1 ratio of the weight of the liquid composition picked up by the fabric to the weight of the dry fabric.

In some embodiments, the padding is carried out at about 80% to about 200% WPU, about 90% to about 175% WPU, about 95% to about 160% WPU, about 100% to about 150% WPU, or about 100% to about 150% WPU. In some embodiments, the padding is carried out at about 80% WPU, about 90% WPU, about 100% WPU, about 110% WPU, about 120% WPU, about 130% WPU, about 140% WPU, about 150% WPU, or about 200% WPU.

In 104, the wetted fabric is heated to yield a pretreated fabric. In some embodiments, the pretreated fabric contains a urethane formed by reaction of the hydrocarbon wax, the crosslinking agent, and the cellulose in the fabric. In some embodiments, the pretreated fabric is a garment (e.g., any article of clothing described herein).

In some embodiments, the wetted fabric is heated in a dryer unit at a temperature greater than a melting temperature of the hydrocarbon wax in the pretreatment composition to yield the pretreated fabric. At this temperature, the hydrocarbon wax melts and diffuses into the fabric and non-covalently bonds to the fabric. A blocked isocyanate crosslinking agent present in the pretreatment composition is unblocked at this temperature and reacts with the carboxyl groups of the oxidized hydrocarbon wax and the hydroxyl groups of the cellulose backbone of the fabric, thus forming a urethane compound and covalently linking the fabric and the hydrocarbon wax. In some embodiments, the temperature in the dryer unit is about 150° C. In some embodiments, the temperature in the dryer unit is in the range of about 100° C. to about 200° C., about 120° C. to about 180° C., or about 140° C. to about 160° C.

The pretreated fabric from 104 may be dried further in 106 to yield a dry pretreated fabric, or may be dyed in 108 with a disperse dye before drying is complete. In some embodiments, the dried fabric in 106 is dyed with a disperse dye in 108. In 110, an article of clothing may be made from the dyed fabric of 108. In some embodiments, the dry pretreated fabric from 106 may be made into an article of clothing in 112, and the article of clothing may be dyed in 114.

In 106, heating is conducted for a period of time that is sufficient to dry the pretreated fabric. In some embodiments, the residual moisture content in the dry pretreated fabric is at most 2 wt. %, at most 1 wt. %, or at most 0.5 wt. %. In some embodiments, the dryer unit is an oven. In some

embodiments, the heating is conducted by drum-drying, tumble-drying, hot air drying, infra-red drying, or hot flue drying.

In 108, the pretreated fabric is dyed using at least one disperse dye. The dyeing process includes contacting the pretreated fabric with a disperse dye to yield the dyed fabric. The dyeing of the treated fabric may be carried out using jet dyeing, carrier dyeing, supercritical carbon dioxide (SCCO<sub>2</sub>) dying or sublimation printing. Jet dyeing may be carried out using jet-dyeing processes and machines that are conventional in the polyester dyeing field. In the jet-dyeing, the treated fabric is dyed at a temperature of about 130° C. In some embodiments, the temperature is in the range of about 100° C. to about 200° C., about 110° C. to about 170° C., or about 120° C. to about 150° C. In some embodiments, the dyeing temperature is sufficient for the disperse dye to diffuse into the hydrocarbon wax. In other embodiments, the dyeing temperature is sufficient for the disperse dye to diffuse into the polyester warp sizing agent. In some embodiments, jet dyeing is followed by scouring the water-dyed fabric at about 40° C. (without an afterclear) to provide the fabric dyed with the disperse dye.

Carrier dyeing may be carried out using carrier solvents used for dyeing polyester fabric. Common polyester dyeing carriers include butyl benzoate, methylnaphthalene, dichlorobenzene, diphenyl and o-phenylphenol. The carrier dyeing is carried out at the boiling point of the carrier solvent for a period of time sufficient to allow the hydrocarbon wax in the pretreated fabric to absorb the carrier and swell, thereby allowing the diffusion of the dye into the hydrocarbon wax. In some embodiments, the carrier drying is followed up by hot air-drying the dyed goods at about 150-180° C.

Supercritical carbon dioxide (SCCO<sub>2</sub>) dying may be carried out under high pressure and elevated temperature conditions at which CO<sub>2</sub> liquefies and solubilizes a disperse dye. The resultant solution of disperse dye in liquid CO<sub>2</sub> may be used to contact the pretreated fabric with a disperse dye, as an alternative to the aqueous disperse dye solutions used in jet dyeing. In some embodiments, SCCO<sub>2</sub> dyeing may be carried out in a stainless steel vessel equipped with a net or a grid for holding a pretreated fabric and a pressure valve. In some embodiments, the vessel is an autoclave. A disperse dye may be placed at the bottom of the vessel, and a pretreated fabric (e.g., dry fabric produced in 106 or wetted fabric produced in 104) may be placed on the net or grid inside the vessel. CO<sub>2</sub> may then be introduced into the vessel in a liquid phase from a cylinder or in a solid form as dry ice. In some embodiments, an amount of dye in the vessel is in a range from about 0.1% o.w.g to about 1% o.w.g. In one example, an amount of dye in the vessel is about 0.4% o.w.g. The vessel may be sealed and heated to a dyeing temperature in a range of about 80° C. to about 140° C., or about 120° C. to about 130° C., at which time CO<sub>2</sub> is isothermally compressed to become a supercritical fluid at a working pressure in the range of about 100 bar to about 350 bar, or about 200 bar to about 250 bar. In some embodiments, the liquor ratio of the pretreated fabric to the SCCO<sub>2</sub> fluid is in the range of about 1:1 to about 1:10. In one example, the liquor ratio is 1:8. In some embodiments, the density of SCCO<sub>2</sub> is about 505 kg/m<sup>3</sup>.

Supercritical fluids are characterized by lower viscosity as compared to common liquid solvents (e.g., water). As a consequence, diffusion processes in SCCO<sub>2</sub> are facilitated, thus promoting uptake of disperse dyes by the pretreated fabric. In some embodiments, contacting the pretreated fabric with SCCO<sub>2</sub> promotes transition of the fabric to a

## 21

rubbery state, lowers the transition glass temperature of the hydrocarbon wax, and promotes diffusion of the disperse dye into the fabric. In some embodiments, the  $\text{SCCO}_2$  dyeing of the pretreated fabric may be carried out for a length of time in the range of about 30 min to about 60 minutes. Upon release of the pressure at the end of the treatment in the supercritical fluid, adsorbed  $\text{CO}_2$  rapidly diffuses out of the fabric. The use of  $\text{SCCO}_2$  instead of water advantageously avoids the step of drying the dyed fabric (e.g., when the pre-treated fabric is jet-dyed in 108), and is an energy efficient and eco-friendly process which does not produce hazardous wastewater. In some embodiments, the  $\text{SCCO}_2$  dyeing is performed without rinsing the dyed fabric with acetone or water after dyeing.

Sublimation printing may be carried out at a sublimation temperature of a disperse dye (e.g., a temperature from about 130° C. to about 210° C.). In some embodiments, sublimation printing is carried out by applying a disperse dye to transfer paper by digital printing, rotogravure technique, or a rotary screen to yield a printed paper. The printed paper is fed into a flatbed heat press machine, where the roller is heated at a temperature up to about 400° F., to transfer the dye from the printed paper to the pretreated fabric. In this process, the fabric is laid onto the printed paper, creating direct contact between the pretreated fabric and the printed paper. The temperature of the heat press machine is approximately the sublimation temperature of a disperse dye. At this temperature, the dye sublimes and transfer to the pretreated fabric to yield the dyed fabric.

In 110, the dyed fabric may be made into an article of clothing.

In 112, the dry pretreated fabric is used to prepare an article of clothing. Any article of clothing conventionally known in the textile industry, such as, for example, underwear (e.g., garments such as bras, panties, hosiery, or camisoles), pants, trousers, khakis, jeans, shirts, shorts, skirts, blouses, tees, tanks, sweaters, dresses, suits, jackets, swimming suits, saris, protective clothing, socks, coats, scarves, footwear, or hats, may be prepared from the treated fabric. Any other article of manufacture that is known to be made from a textile material can also be prepared from the pretreated fabric. In 114, the article of clothing prepared from the pretreated fabric may be dyed with at least one disperse dye as described herein with respect to dyeing of a pretreated fabric to yield a dyed article of clothing.

#### Fabric Treatment with Disperse Dye-Containing Compositions

FIG. 2 is a flow chart showing operations in exemplary process 200 for treating fabric with a disperse dye-containing composition. In 202, a fabric is contacted with a composition including a pretreatment composition and a disperse dye to yield a wetted treated fabric. In some embodiments, the wetted treated fabric contains particles of disperse dye adsorbed on the surface of the fabric. In some embodiments, the fabric is a garment.

In some embodiments, treating the fabric with a liquid disperse dye-containing composition is carried out using any one of the padding protocols described herein with respect to pretreating the fabric with the pretreatment composition. In some embodiments the treating is carried out at about 100% WPU. In one example, when the fabric is a garment, the dye-containing composition may be applied to the garment using mist and tumble method at about 100% WPU.

In 204, the wetted treated fabric is heated to yield a treated fabric. The treated fabric contains a urethane formed by a reaction of the hydrocarbon wax, the crosslinking agent, and cellulose in the fabric. The disperse dye remains adsorbed on

## 22

the surface of the treated fabric during heating. Heating of the wetted fabric removes about 60-80 wt. % of water from the wetted fabric.

In 206, the wetted treated fabric is dried at a temperature above the melting point of the hydrocarbon wax to yield the dry treated fabric. The drying may be carried out as described herein with respect to the pretreated fabric.

In some embodiments, the drying of the wetted treated fabric is carried out in several steps. In one example, the 10 wetted fabric is dried using a hot flue air dryer, infrared (IR) radiation, or a combination thereof. This first drying step results in the removal of about 60-80 wt. % of water from the wetted treated fabric. In the following drying step, the padded fabric is dried using heated cylinders or the fabric is 15 thermosoled in the first zones of the tenter frame around 150° C. to yield the dry treated fabric. In one example, when the fabric is a garment, the wetted treated garment is tumble dried at about 150° C. In some embodiments, the disperse dye remains adsorbed on the surface of the fabric throughout 20 drying. In some embodiments, the residual moisture content in the dry treated fabric is at most 2 wt. %, at most 1 wt. %, or at most 0.5 wt. %. In some embodiments, the dry treated fabric contains a urethane compound formed by reaction of a hydrocarbon wax, a crosslinking agent, and cellulose in the 25 fabric. The urethane compound is formed as described herein with respect to the pretreatment of fabric with a pretreatment composition. In some embodiments, the disperse dye remains adsorbed on the surface of the dry treated fabric.

In 208, the dry treated fabric is thermosoled to yield a dyed fabric. As used herein, the term "thermosol" refers to a process of contacting a dry fabric with a disperse dye at a temperature that is higher than the sublimation temperature of the disperse dye.

In some embodiments, the dry treated fabric is thermosoled by contacting the dry treated fabric with a hot metal surface, or by contacting the dry treated fabric with hot air at a temperature in the range of about 190° C. to about 210° 35 C., for a time period from about 30 seconds to about 5 min, or from about 1 min to about 2 min. In some embodiments, the fabric is thermosoled for about 90 seconds. In one example, when the fabric is a garment, the dry treated garment may be garment cured for about 90 seconds at about 210° C. In the garment curing process, the garment is placed 40 in an insulated oven at a temperature above the sublimation temperature of a disperse dye, such that the dye sublimes into the fabric. In some embodiments, during a thermosol process, when the dry treated fabric is heated at or above the sublimation temperature of the disperse dye, the disperse 45 dye sublimes and the hydrocarbon wax absorbs the dye vapor. The dye diffuses into the hydrocarbon wax, thereby coloring the fabric. In some embodiments, the thermosoled dyed fabric is scoured at about 40° C. (without an afterclear) to provide the fabric dyed with the disperse dye.

In 210, the dyed fabric may be made into an article of clothing.

## EXAMPLES

60 Materials and Methods  
Chemical Compounds  
Turpex ACN (polyethylene wax) and Thermocol MP (anti-migrating agent) were purchased from Huntsman. Fadex ECS (UV absorber) was purchased from Archroma. 65 PW 600 polyester warp sizing agent was purchased from Ulterion. Ruco-Coat FX 8041 (urethane crosslinking agent) was purchased from Rudolf Chemie. Polyethylene wax,

23

anti-migrant, UV absorber, polyester warp sizing agent, and urethane crosslinking agent were obtained as aqueous emulsions. Various disperse dyes were purchased from numerous commercial suppliers.

## Fabric

Cotton fabric (greige or bleached) was used in the experiments.

## Example 1

Fabric Pretreatment for Conventional and Supercritical CO<sub>2</sub> Disperse Dyeing

## Preparation of the Fabric Pretreatment Composition:

In the pretreatment bath, water (885 mL) was added. Agitation was started, followed by the slow addition of an aqueous dispersion of Ruco-Coat FX 8041 (15 g), an aqueous emulsion of Turpex ACN (50 g), and an aqueous dispersion of Ulterion PW-600 to the pretreatment bath.

## Pretreatment of Fabric for Dyeing with Disperse Dyes:

The pretreatment dispersion was added to the pad liquor trough. The composition was padded onto fabric at 100% wet pick-up. The padded fabric was bone dried in an oven at 150° C.

## Example 2

## Disperse Dyeing of Pretreated Fabric

The pretreated fabric of Example 1 was loaded into a jet dye machine, a SCCO<sub>2</sub> dye machine, or used as a base for sublimation printing. The fabric was dyed with Disperse Blue 79 and Fadex ECS using standard procedures around 130° C. The water dyed fabric was scoured at 40° C., without an afterclear to remove surface dye. The dyed fabric was unloaded from the machine.

## Example 3

## Fabric Treatment for Thermosol Disperse Dyeing

## Preparation of the Fabric Treatment Composition:

In the treatment bath, water was added. Agitation was started, followed by the slow addition of an aqueous dispersion of Ruco-Coat FX 8041 (15 g), an aqueous emulsion of Turpex ACN (50 g), Thermocol (10 g), an aqueous dispersion of Ulterion PW-600, Fadex ECS (25 g), and Disperse Blue 79 to the treatment bath. The amount of water was used such that the total amount of liquid was 1 L.

## Thermosol Dyeing of Fabric with Disperse Dyes:

The treatment dispersion was added to the pad liquor trough. The composition was padded onto knitted fabric at 100% wet pick-up. The treated fabric was dried in the thermosol apparatus in the first zones of the tenter frame around 150° C. The dry treated fabric was thermosoled for 90 seconds at 210° C. The water dyed fabric was scoured at 40° C., without an afterclear to remove surface dye. The dyed fabric was unloaded from the machine.

## Thermosol Dyeing of Garment with Disperse Dyes:

A garment (e.g., a knitted t-shirt) was treated with the treatment composition using the mist and tumble procedure at 100% wet pick up. The treated garment was tumble dried and then thermosol cured for 90 seconds at 210° C. The dyed garment was scoured at 40° C., without an afterclear. The dyed fabric was unloaded from the machine.

24

## Example 4

## Properties of the Dyed Fabric

5 The efficiency of the compositions and methods of Examples 1-3 for dyeing the cotton fabric with disperse dyes was evaluated using AATCC Test Method 60-2A Washfastness.

## 10 Other Embodiments

It is to be understood that while the present application has been described in conjunction with the detailed description thereof, the foregoing description is intended to illustrate and not limit the scope of the present application, which is defined by the scope of the claims. Other aspects, advantages, and modifications are within the scope of the following claims.

20 What is claimed is:

1. A liquid fabric treatment composition comprising: a hydrocarbon wax; a crosslinking agent; and a polyester warp sizing agent, wherein the polyester warp sizing agent is anionic and comprises sulfate moieties.
2. The composition of claim 1, wherein the composition is an aqueous dispersion.
3. The composition of claim 1, wherein the hydrocarbon wax comprises polyethylene wax.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700

**25**

16. A method of treating fabric, the method comprising: contacting fabric comprising cellulose with a liquid dispersion to yield a pretreated fabric, wherein the liquid dispersion comprises:  
 a hydrocarbon wax;  
 a crosslinking agent; and  
 a polyester warp sizing agent; and  
 heating the pretreated fabric to yield a treated fabric, wherein the treated fabric comprises a urethane formed by a reaction of the hydrocarbon wax, the crosslinking agent, and the cellulose.
17. The method of claim 16, further comprising dyeing the treated fabric with a disperse dye.
18. The method of claim 16, wherein the liquid dispersion comprises a disperse dye.
19. A liquid fabric treatment composition comprising:  
 a hydrocarbon wax;  
 a crosslinking agent;  
 an ultraviolet light inhibitor; and  
 a polyester warp sizing agent.

**26**

20. A liquid fabric treatment composition comprising:  
 a hydrocarbon wax;  
 a crosslinking agent comprising a nonionic blocked isocyanate; and  
 a polyester warp sizing agent, wherein the liquid fabric treatment composition is an aqueous dispersion.
21. A liquid fabric treatment composition comprising:  
 a hydrocarbon wax;  
 a crosslinking agent comprising a nonionic blocked isocyanate; and  
 a polyester warp sizing agent,  
 wherein the crosslinking agent reacts with the hydrocarbon wax and a cellulose-containing fabric to form a urethane.
22. A liquid fabric treatment composition comprising:  
 a hydrocarbon wax;  
 a crosslinking agent comprising a nonionic blocked isocyanate;  
 an anti-migrant; and  
 a polyester warp sizing agent.

\* \* \* \* \*